

## UNITED STATES PATENT OFFICE

2,033,196

## EXPLOSIVE COMPOSITION

Norman G. Johnson and Harold A. Lewis, Woodbury, N. J., assignors to E. I. du Pont de Nemours & Company, Wilmington, Del., a corporation of Delaware

No Drawing. Application April 21, 1933,  
Serial No. 667,229

8 Claims. (Cl. 52—13)

This invention relates to pulverulent dynamite compositions and more particularly to such compositions containing only a relatively small amount of sensitive liquid ingredient, but yet sufficient of such liquid ingredient that the hazard of mixing and handling a dusty composition is not present.

The commercial high explosives of the dynamite type, for the most part, contain nitroglycerin as the sensitive explosive ingredient, which causes the dynamites to detonate invariably under the influence of a commercial blasting cap and to propagate the explosion throughout the dynamite, after detonation has been once initiated. In recent years, the tendency has increasingly been to replace nitroglycerin by ammonium nitrate as far as possible because of various advantages obtained, the replacement being limited, however, by the necessity of maintaining the proper degree of sensitiveness to detonation and propagation.

Nitroglycerin dynamites have been used with considerable satisfaction over a long period of years, and no other explosive material has been available that possessed the generally desirable properties of this compound as the desired sensitized ingredient. Nitroglycerin, however, has one objectionable property that has been a draw-back to its use, namely, that of causing severe headaches in the case of persons coming in contact with it, or breathing its vapors. This toxic property is possessed not only by nitroglycerin, but by all the aliphatic liquid nitric esters.

Various explosives have been suggested and used on a limited scale which consisted of all solid ingredients, and such explosives have been free from the undesirable physiological effects produced by nitroglycerin and explosives containing it. The various nitrostarch dynamites are one example of such explosives and have had considerable use in America. Nitrostarch, however, is a material relatively insensitive to detonation, and considerable difficulty has been encountered in producing uniformly sensitive and satisfactory explosives of this type. Moreover, it is an amorphous material, dusty in nature, so that there is a certain degree of hazard connected with the mixing and handling of such explosives. Nitrostarch also is of a lower order of stability than nitroglycerin, so much so that its use has never been approved in European explosives.

The object of our invention is to provide an improved explosive composition free from headache-producing properties. A further object is such an explosive, the sensitiveness of which is uniform

and can be readily controlled within the desired limit. A still further object is an explosive consisting essentially of solid ingredients, but one which is not dusty in nature and not unduly sensitive to shock. Further objects will present themselves as the description of the invention proceeds.

The foregoing objects are accomplished, according to our invention, by the production of a pulverulent dynamite composition containing pentaerythritol tetranitrate and a relatively small amount of a liquid ingredient. While the use of any liquid will be advantageous in reducing the dusty nature of such solid explosives, it is essential for our purpose that a non-volatile liquid be employed in order that no change in composition may take place in the explosive during storage. Water is not a suitable liquid for this use because of its solvent and hydration effects on various inorganic ingredients that may be present in the explosive composition.

Preferably ammonium nitrate will be an ingredient of the explosive composition according to our invention, along with the pentaerythritol tetranitrate. Ammonium nitrate is economically available and possesses great strength as an explosive when present with satisfactory sensitizing agents, and for these reasons is a desirable component. Pentaerythritol tetranitrate in such explosive compositions not only acts as a very powerful explosive itself, but serves also as a sensitizer and booster in bringing about the complete detonation of the ammonium nitrate at its maximum strength.

As stated previously, various non-volatile and non-aqueous liquids may be used in our explosive compositions with the object of reducing the dusty nature of the pulverulent mixtures. For example, we may employ a non-volatile oil, such as engine oil. Also, a relatively small amount of a non-volatile liquid aromatic nitrocompound may be used, such as, for example, liquid dinitrotoluene. We may also incorporate in the explosive composition an aliphatic liquid nitric ester of a polyhydroxy alcohol. Nitroglycerin is the preferred liquid compound of this class, and it is this type of explosive which we find most valuable.

The choice of liquid ingredient in the explosive compositions will affect the proportions of other ingredients present. If engine oil or other petroleum hydrocarbon is used, this ingredient has a marked desensitizing effect and a higher percentage of sensitive explosive material, such as pentaerythritol tetranitrate will then be necessary. If nitroglycerin is present, on the other hand, it

will be possible to use a decreased amount of pentaerythritol tetranitrate and a correspondingly larger percentage of ammonium nitrate, and still obtain a satisfactory degree of sensitiveness. In 5 such a composition nitroglycerin will be the primary sensitizing agent. Liquid dinitrotoluene and other liquid aromatic nitrocompounds are intermediate, with respect to sensitizing effect, between the two types of liquids previously discussed. Preferably we use the liquid ingredient 10 of our explosives in an amount between 0.2 and 5.0%. The use of less than 5% of engine oil for example is desirable, since a larger amount would make the explosive composition too insensitive to 15 detonation and propagation. In the case of liquid aliphatic nitric esters, the use of not more than 5% has the advantage that the explosive thus obtained is essentially a non-headache dynamite because of the small percentage of liquid 20 nitric ester present. Less than 0.2% of liquid is undesirable, since such small amounts do not have the desired effect on the properties of the explosive.

As previously stated, ammonium nitrate will 25 preferably be included in our explosive compositions. Similarly, sodium nitrate may be present in its usual capacity as oxidizing agent, as well as carbonaceous combustible ingredients, acid-accepting materials, and other customary constituents of dynamite compositions.

30 The following examples are illustrative of compositions made according to our invention, containing pentaerythritol tetranitrate and the three types of liquids described in the foregoing:

|                                    | I     | II    | III   |
|------------------------------------|-------|-------|-------|
| Pentaerythritol tetranitrate       | 35.0  | 12.0  | 16.0  |
| Engine oil                         | 0.5   |       |       |
| Liquid dinitrotoluene              |       | 2.0   |       |
| Nitroglycerin                      |       |       | 3.0   |
| 40 Ammonium nitrate                |       | 66.5  | 50.0  |
| Sodium nitrate                     | 56.0  | 10.0  | 21.0  |
| Sulfur                             | 5.0   |       |       |
| Carbonaceous combustible materials |       | 9.0   | 9.5   |
| Chalk                              | 3.5   | 0.5   | 0.5   |
|                                    | 100.0 | 100.0 | 100.0 |

45 In the above examples, I represents a composition containing pentaerythritol tetranitrate with engine oil as the dust-reducing liquid, no ammonium nitrate being present. II and III are examples of powders containing pentaerythritol tetranitrate and ammonium nitrate, liquid dinitrotoluene and nitroglycerin being the liquids present, respectively.

50 We are aware of the fact that pentaerythritol tetranitrate has been used heretofore in explosive compositions. Von Herz, for example, discloses (in British Patent 11,809 of 1913) safety explosive compositions containing ammonium nitrate in which PETN was present. His compositions, however, contained solid ingredients only and did not include any liquid ingredient such as is present in our compositions and which is advanta-

geous in reducing the hazard of dustiness during mixing and handling, and which gives a beneficial sensitizing effect, when nitroglycerin or other similar liquid nitric ester is employed.

5 Pentaerythritol tetranitrate compositions have been disclosed by Stettbacher also, and U. S. Patent 1,867,287, for example, illustrates his compositions. Stettbacher, however, was considering plastic explosives only, and his invention was directed to such compositions. A plastic mixture 10 was obtained by the combined use of nitroglycerin and pentaerythritol tetranitrate in varying proportions, and these plastic mixtures were then diluted with oxidizing agents and other ingredients. A plastic mixture was maintained 15 throughout, and such explosives are quite different from the pulverulent dynamites of the present application.

Our invention has been described in detail in 20 the foregoing, but it will be apparent that various departures may be made from the specific compositions disclosed in the foregoing example. While nitroglycerin has been employed as the liquid nitric ester, it will be understood that we may substitute for this various other liquid aliphatic 25 nitric esters such as ethyl nitrate, ethylene glycol dinitrate, nitrated chlorhydrins, tetranitrodiglycerin and the like.

We intend, therefore, to be limited only as indicated in the following patent claims. 30

We claim:

1. A pulverulent high explosive composition, comprising pentaerythrite tetranitrate and a relatively small amount of a non-volatile liquid aromatic nitrocompound. 35

2. A pulverulent high explosive composition, comprising pentaerythrite tetranitrate and a relatively small amount of liquid dinitrotoluene.

3. A pulverulent dynamite composition, comprising pentaerythrite tetranitrate and a relatively small amount of a non-volatile liquid nitric ester. 40

4. A pulverulent dynamite composition, comprising pentaerythrite tetranitrate and a liquid nitric ester of a polyhydroxy alcohol in the amount of 0.2 to 5.0%. 45

5. A pulverulent dynamite composition, comprising pentaerythrite tetranitrate, at least one inorganic oxidizing agent, and a liquid nitric ester of a polyhydroxy alcohol in the amount of 0.2 to 50 5.0%.

6. A pulverulent dynamite composition, comprising pentaerythrite tetranitrate and 0.2 to 5.0% nitroglycerin.

7. A pulverulent dynamite composition, comprising pentaerythrite tetranitrate, ammonium nitrate, carbonaceous combustible material, and 0.2 to 5.0% of nitroglycerin. 55

8. A pulverulent dynamite composition comprising pentaerythrite tetranitrate and a liquid nitrated organic compound. 60

NORMAN G. JOHNSON.  
HAROLD A. LEWIS.